

Dec. 26, 1950

T. R. THOMPSON  
PHOTOGRAPHIC EMULSIONS CONTAINING  
TRINUCLEAR CYANINE DYES  
Filed April 30, 1949

2,535,995



Fig. 1.



Fig. 2.



Fig. 3.



INVENTOR  
Thomas R. Thompson

BY *Henry B. Elling*  
*Henry B. Elling*  
ATTORNEYS

## UNITED STATES PATENT OFFICE

2,535,995

PHOTOGRAPHIC EMULSIONS CONTAINING  
TRINUCLEAR CYANINE DYES

Thomas R. Thompson, Binghamton, N. Y., assignor to General Aniline & Film Corporation, New York, N. Y., a corporation of Delaware

Application April 30, 1949, Serial No. 90,711

4 Claims. (Cl. 95—7)

1

This invention relates to photographic gelatinous silver-halide emulsions, and more particularly, to photographic emulsions sensitized by means of new trinuclear cyanine dyes containing a terminal 5-membered nitrogenous heterocyclic ring system.

The use of sensitizing dyes, particularly in multilayer color film, poses many problems. It is known that sensitizing dyes operate by dyeing the silver-halide grain. To do this, they must be adsorbed to the silver-halide. If they are displaced from the silver-halide grains, they lose their effectiveness as sensitizers. It is also known that many color formers used in color photography have greater affinity for silver-halides than the sensitizers, and act to displace the same from the silver-halide grains. One must, therefore, select a sensitizer which will not be so displaced.

Another problem arises as regards the migration of the sensitizers from one emulsion to another. Where this ensues, color distortion is the inevitable result. Many proposals have been made dealing with the anchoring of compounds in silver-halide emulsions, the most noteworthy being the use of a long alkyl chain (see Wilmanns et al., United States Patent 2,186,849).

It is, therefore, necessary when providing sensitizers particularly for color photography, to make certain that they have (1) the proper sensitizing power, (2) the ability to withstand displacement from silver-halide grains by color formers, and (3) the ability to resist diffusion from one sensitized emulsion to another.

Efforts which satisfy the last prerequisite, unfortunately, often lead to compounds which will not meet the first two tests. Thus, it is known that the sensitizing power of cyanine dyes varies with the substituent on the cyanine N-atoms. Where this substituent is alkyl, the power decreases as the chain length increases. Hence, if a long alkyl chain be used to anchor the dye in the emulsion, we end up with a product of little or no sensitizing power. The use of other expedients to anchor the dye, on the other hand, often gives products incapable of withstanding the displacement action of color formers insofar as the silver-halide grains are concerned. It is thus manifest that the provision of sensitizers having the necessary prerequisite is a difficult problem, to say the least.

It is known that many cyanine dyes sensitize photographic silver-halide emulsions to high red sensitivity. Most of these dyes, however, are not suitable for sensitizing silver-halide emulsions

2

containing color coupling components. This is thought to be due to a physical displacement which the sensitizing dye undergoes when color coupling components are added. That is, the sensitizer is adsorbed to the surface of the silver-halide grain, and then, with addition of color coupling component, is displaced therefrom. Moreover, most of the cyanine dyes are incompatible with silver-halide emulsion stabilizers, such as, for example, mercapto-substituted tetrazoles.

An object of the present invention is to provide photographic silver-halide emulsions with trinuclear sensitizing dyestuffs containing a terminal 5-membered nitrogenous heterocyclic ring system.

A further object is to provide such dyes which are free from the disadvantages noted above.

Other objects and advantages of this invention will become apparent by reference to the following specification in which its preferred details and embodiments are described.

This invention is based on the discovery that trinuclear cyanine dyes containing a terminal 5-membered ring system not only sensitize a photographic silver-halide emulsion to high red sensitivity, but are also compatible with color coupling components for the cyan dye image and with practically all emulsion stabilizers including the mercapto-substituted tetrazoles. In the latter combination the sensitizing action of the dyes is not impaired nor diminished. In addition to these desirable characteristics, it has been further found that when the dyes are used in conjunction with color coupling components for the blue-green image, the spectral curves of these dyes show a desirable gap in the green region of the spectrum, i. e., the dye sensitivity is more selective to the red spectral region. The sensitizing capacity of these dyes is not only maintained in the presence of color coupling components for the blue-green image, especially those components containing long alkyl chains, but is in part rendered more selective.

Some of the trinuclear cyanine dyes of this invention, which sensitize emulsions to the regions of longer wavelengths, are of extreme value in the manufacture of infrared silver-halide emulsions which can be exposed through light yellow filters instead of the ordinarily used heavy gray filters in view of their low sensitizing power for the green, yellow and red. An additional advantage of these dyes is their ability to remain fixed in the layer in which they are originally deposited.

The trinuclear cyanine dyes fulfilling the above

advantage are obtained in excellent yield and in readily purifiable form by treating a 3-alkyl, 3-aryl, or 3-aralkyl substituted 5-membered ketomethylene heterocyclic compound containing a reactive methylene group adjacent to a keto group of the type commonly employed in merocyanine dyes with a thiazolone cyanine dye salt intermediate in the presence or absence of a suitable solvent, such as an aliphatic alcohol, e. g., methyl, ethyl, n-propyl, isopropyl, and the like, and in the presence of a basic condensing agent, such as trimethylamine, triethylamine, pyridine, methylpyridine, ethylpyridine, quinoline, potassium carbonate and the like, on a steam bath or by heating the reaction mixture at reflux for a period of from 5 to 20 minutes.

The dyes obtained by the foregoing procedure are characterized by the following general formula:



wherein R represents hydrogen or an alkyl group, e. g., methyl, ethyl, propyl or butyl, R being only alkyl when m represents 1, R<sub>1</sub> and R<sub>2</sub> which may be alike or different represent an alkyl, allyl, aryl, or aralkyl group, e. g., methyl, ethyl, propyl, phenyl, naphthyl, tolyl, benzyl, phenethyl and the like, R<sub>3</sub> represents an aliphatic, aryl, aralkyl or substituted group of this type, e. g., methyl, ethyl, propyl, butyl, hydroxyethyl, ethoxyethyl, phenyl, tolyl, naphthyl, benzyl, phenethyl, mephthyl and the like, m represents a positive integer of from 1 to 3, X represents an acid radical, e. g., chloride, bromide, iodide, or alkyl sulfate, alkyl p-toluenesulfonate or perchlorate, Y represents the residue of a 5-membered heterocyclic nitrogenous ring system of the type used in merocyanine dyes, e. g., N-alkyl, N-allyl, N-aryl, N-aralkyl substituted derivatives of rhodanic acid, 5-pyrazolones, thiazolediones, thiazolones, oxazolediones, thiohydantoins, and the like, and Z represents the residue of a heterocyclic nitrogenous nucleus of the type used in cyanine dyes, e. g., oxazoles, thiazoles, selenazoles, and their polycyclic homologues, such as those of the benzene, naphthalene, acenaphthene, and anthracene series, pyridine, and its polycyclic homologues, such as quinoline and  $\alpha$ - and  $\beta$ -naphthoquinolines, perinaphthiazoles, indolenines, diazines, such as pyrimidines, and quinazolines, diazoles (e. g., thio- $\beta$ - $\beta$ -diazole), oxazolines, pyrrolines, thiazolines and selenazolines (the polycyclic compounds of these series being substituted if desired in the carbocyclic rings with one or more conventional groups, such as alkyl or aryl, as below, amino, hydroxy, alkoxy, i. e., methoxy, ethoxy, etc., and methylene-dioxy groups, or by halogen atoms, i. e., chlorine or bromine, etc.).

The N-substituted 5-membered ketomethylene heterocyclic compounds of the type commonly employed in merocyanine dye syntheses, which are treated with a thiazolone cyanine dye intermediate are characterized by the following general formula:



wherein Y and R<sub>1</sub> have the same values as above.

As typical examples of such compounds, the following may be mentioned:

- 3-ethylrhodanine
- 3-allylrhodanine
- 3-phenylrhodanine
- 3-benzylrhodanine
- 3-methyl-4-keto-2-seleno - tetrahydro - oxazole
- 3-phenyl-4-keto-2-seleno-tetrahydro-selenazole
- 3-propyl-4-keto-2-seleno - tetrahydro - thiazole
- 1-phenyl-3-methyl-5-pyrazolone
- 1-methyl-5-pyrazolone
- 1,3-dimethyl-5-pyrazolone
- 1,3-diphenyl-5-pyrazolone
- 3-phenyl-2,4-thiazoledione
- 2-diphenylamino-3-ethyl-4(5)-thiazolone
- 3-ethyl-2-thio-2,4(3,5)-oxazoledione
- 3-ethyl-1-phenyl-2-thiohydantoin, and the like.

The thiazolone cyanine dye intermediates utilized as the coreactants with the foregoing N-substituted 5-membered ketomethylene heterocyclic compounds, are characterized by the following general formulae:



and



wherein R<sub>2</sub>, R<sub>3</sub>, X and Z have the same values as above, R<sub>4</sub> represents an aryl group of the benzene and naphthalene series such as phenyl, chlorophenyl, diphenyl or naphthyl, R<sub>5</sub> represents either hydrogen or an acetyl group, R<sub>6</sub> represents an alkyl or aralkyl group, e. g., methyl, ethyl, propyl, isopropyl, benzyl,  $\beta$ -phenethyl, and the like, R<sub>7</sub> represents an alkyl group, e. g., methyl, ethyl, propyl, isopropyl, butyl, isobutyl, etc., and n represents a positive integer of from 1 to 3, and W represents the atoms necessary to complete a saturated nitrogenous heterocyclic nucleus, such as, for example, piperidine,  $\beta$ - and  $\gamma$ -piperidine, pyrrolidine, morpholine, tetrahydroquinoline, and the like.

The dyestuff intermediates illustrated by the Formulae a and c are prepared according to the method described in my copending application Serial No. 66,571, filed on December 21, 1948, and the intermediates illustrated by the second Formula b are prepared according to the method described in my copending application Serial No. 66,572, filed on December 21, 1948.

The dyestuff intermediates illustrated by Formula a are, in general, obtained by treating a diarylformamidine or its vinyllog such as  $\beta$ -ani-

linoacrolein anil hydrochloride or glutaconic aldehyde dianil hydrochloride, in the presence of an acid condensing agent, such as acetic anhydride or in the presence of a basic condensing agent, such as triethylamine or piperidine, with a thiazolone cyanine dye.

The dyestuff intermediates illustrated by Formula *b* are obtained by treating a triazolone cyanine dye with an aliphatic acid anhydride in the presence of a mixture of pyridine and triethylamine followed by treatment with phosphorous pentasulfide to yield the thioether derivative which is subsequently alkylated with an alkylating agent in the usual way to yield the thioether derivative.

The dyestuff intermediates containing a terminal saturated heterocyclic nitrogenous ring nucleus are prepared by treating a thiazolone cyanine dye with a diarylformamidine or its vinyllog in the presence or absence of an aliphatic alcohol as a diluent and in the presence of a saturated heterocyclic nitrogenous compound, such as morpholine, piperidine, tetrahydroquinoline, and the like.

The thiazolone cyanine dyes utilized in preparing the foregoing intermediates are characterized by the following general formula:



wherein  $\text{R}_2$ ,  $\text{R}_3$ ,  $\text{X}$  and  $\text{Z}$  have the same values as above, and are prepared according to the method described in my copending application Serial No. 786,814, filed November 18, 1947. In general, the method consists of condensing a substituted thioamide with an  $\alpha$ -halogen acetic acid. The compounds, in view of their ketomethylene configuration undergo keto-enol tautomerism, i. e., the keto group enolizes to form a hydroxyl group.

The following examples describe the preparation of some of the thiazolone cyanine dye intermediates illustrated by Formulae *a* and *b* which are utilized in the preparation of the trinuclear cyanine dyes.

#### Example I



A mixture of 5 grams of diphenylformamidine, 5 grams of the thiazolone cyanine dye of the following structure:



and 15 cc. of acetic anhydride was heated at 140° C. for 30 minutes. After cooling, the prod-

uct was precipitated with ether and purified by dissolving in a small amount of methanol followed by precipitation with ether. A yield of 5.9 grams of yellow green crystals, having a melting point at 213–215° C., was obtained.

#### Example II



A mixture of 75 cc. of pyridine, 15 cc. of propionic anhydride, 15 cc. of triethylamine, and 15 grams of the thiazolone cyanine dye of the following structure:



was heated at 120° C. for 30 minutes. Fifteen grams of phosphorus pentasulfide were added in portions and the reaction mixture stirred at 120° C. for 30 minutes. The product was isolated by pouring the reaction mixture into 300 cc. of water. The product was purified by washing with water and subsequently grinding with acetone. A yield of 10.9 grams of yellow glistening crystals melting at 255–260° C. was obtained. The product was fused with 10 cc. of methyl sulfate at 95° C. for 10 minutes to yield a thick solution which upon treatment with an acetone solution of sodium iodide deposits yellow crystals.

#### Example III



A mixture of 75 cc. of pyridine, 10 cc. of propionic anhydride, 10 cc. of triethylamine, and 13 grams of the thiazolone cyanine dye of the following structure:



was heated with stirring at 120° C. for 20 minutes. During the course of 10 minutes, a total of 10 grams of phosphorus pentasulfide was added in portions at 120° C. After an additional 10 minutes heating and stirring at 120° C., the mixture was poured into cold water and stirred until the first formed oil solidified. The crude

product was stirred with 300 cc. of a 1% aqueous solution of sodium hydroxide and purified by boiling out with isopropanol. There was obtained 10.2 grams of yellow powder which decomposes at about 200° C.

A mixture of 9.3 grams of the yellow powder and 10 grams of methyl p-toluenesulfonate was fused at 95° C. for 1 hour. After cooling, the product was washed with ether and dissolved in 10 cc. of warm acetone. The final product was

10



precipitated as the iodide, by adding 25 cc. of methanol containing 20% sodium iodide. The product was washed with water and purified by boiling out with isopropanol. A yield of 4.3 grams of a product melting at 225-228° C. was obtained.

*Example IV*



A mixture of 15 cc. of pyridine, 2 cc. of propionic anhydride, 2 cc. of triethylamine, and 2.0 grams of the thiazolone cyanine dye of the following structure:



was heated at 120° C. for 3 minutes. There were then added 2 grams of phosphorus pentasulfide and the mixture heated at 115° C. for 15 minutes. A dark red oil was precipitated by the addition of 100 cc. of water and washed with water by decantation. The product was fused with 3 cc. of methyl sulfate at 95° C. for 10 minutes to yield 4.5 grams of a yellow-orange solution which may be employed in dye synthesis.

*Example V*



A mixture of 0.5 gram of the product of Example III, 0.3 gram of  $\beta$ -anilinoacrolein anil hydrochloride, 10 cc. of methanol, and 0.5 gram

of piperidine was heated at reflux for 5 minutes. The reaction mixture was poured into 60 cc. of water containing 1 gram of potassium iodide. The crystals were separated and purified by boiling out with isopropyl alcohol. A yield of 0.4 gram of a product having a melting point of 270-271° C. was obtained. A methanol solution of the compound has an absorption maximum at 540 m $\mu$ .

*Example VI*



20 A mixture of 2.85 grams of glutaconaldehyde dianil hydrochloride, 4.3 grams of the compound of Example III, 1 cc. of piperidine and 50 cc. of methanol was heated at reflux for 30 minutes. The reaction mixture was poured into 300 cc. of water containing 5 grams of potassium iodide. The precipitated product was filtered and boiled out with isopropyl alcohol. A yield of 3.7 grams of a compound having a melting point of 195-198° C. was obtained. A methanol solution of the product has an absorption at 624 m $\mu$ .

The anions of the foregoing thiazolone cyanine dye salts may be replaced by other anions, such as iodide, thiocyanate or perchlorate ions by treating an alcohol solution of the halogen salt with an aqueous or aqueous-alcohol solution containing a sodium or potassium salt of the desired anion.

The following examples describe in detail the improved and simplified method of preparing tri-nuclear cyanine dyes from the foregoing thiazolone cyanine dye intermediates, but it is to be understood that they are given merely for the purpose of illustration and are not to be construed as limitative.

*Example VII*



50 A mixture of 0.35 gram of 3-allylrhodanine, 0.8 gram of the intermediate of Example I, 50 cc. of methanol, and 0.5 cc. of triethylamine was heated at reflux for 5 minutes. The crude dye was boiled out with methanol and finally crystallized from pyridine. A yield of 1.25 grams of a product melting above 295° C. was obtained. The absorption maximum of this dye in a methanol solution is 610 m $\mu$ .

*Example VIII*



A mixture of 0.35 gram of 3-allylrhodanine, 1.03 grams of the intermediate of Example III, 50 cc. of methanol and 1 cc. of triethylamine was heated at reflux for 15 minutes. After cooling, the dye was separated and purified by boiling out with methanol. A yield of 0.5 gram of a product melting at 173-175° C. was obtained. The absorption maximum in methanol is 594 m $\mu$ . When the dye is incorporated into a photographic emulsion the sensitization maximum is 650 m $\mu$ .

*Example IX*



A mixture of 0.6 gram of the intermediate of Example V, 0.2 gram of 3-methyl-1-phenylpyrazolone, 20 cc. of methanol, and 1 cc. of triethylamine was heated at reflux for 10 minutes. The very slightly soluble dye was filtered off and purified by boiling out with methanol. A yield of 0.6 gram of the purified dye was obtained.

*Example X*



A mixture of 1.2 grams of the intermediate of Example VI, 0.5 gram of 3-allyl-1-methyl-2-thiohydantoin, 25 cc. of methanol and 1 cc. of triethylamine was heated at reflux for 5 minutes. After cooling the dye crystals were removed and purified by boiling out with methanol. A yield of 0.5 gram of a product melting at 199-203° C. was obtained. The absorption maximum in methanol is 621 m $\mu$ . The sensitization of a photographic emulsion is extended to 720 m $\mu$  with a maximum at 680 m $\mu$ .

*Example XI*



A mixture of 0.5 gram of the product of Example II, 0.2 gram of 3-allylrhodanine 15 cc. of isopropyl alcohol, and 0.5 cc. of triethylamine was heated at reflux for 10 minutes. The dye separated on cooling and was purified by boiling out with isopropyl alcohol. A yield of 0.4 gram of the dye was obtained. The absorption maximum of a methanol solution is 583 m $\mu$ . When incorporated in a photographic emulsion the maximum sensitization is at 640 m $\mu$ .

The diagrammatic spectrograms constituting the accompanying drawing illustrate the regions of the spectrum to which some of the trinuclear cyanine dyes will sensitize a gelatino silver-

halide emulsion containing about 4-5% of silver-halide and the extent of the sensitization at various wavelengths. Figures 1 to 3 of this drawing illustrate the sensitizing properties of the dyes prepared in accordance with Examples VIII, X, and XI, respectively.

This application is a continuation-in-part of my copending application Serial No. 66,574, filed December 21, 1948, now Patent No. 2,513,730.

10 While the present invention has been described in considerable detail with reference to certain preferred procedures and materials employed, it is understood that the improved process of preparing trinuclear cyanine-dyes is not limited thereto, and that numerous variations and modifications described in the foregoing specification may be made as, for example, the dyes which contain a thioketone group in the terminal 5-membered heterocyclic nitrogenous nucleus, as illustrated 15 in Examples VII, VIII, X, and XI, may be further treated with a quaternizing compound such as methyl iodide. The quaternized compound is then condensed under reflux conditions with a cyclammonium base or salt of the type used in cyanine dyes, such as 2-methylbenzothiazole 20 ethiodide and the like, having a reactive methyl group in *a*-position to the nitrogen atom thereof, in the presence of a basic condensing agent such as pyridine. In the first reaction (alkyla-



tion), the trinuclear dye is modified to the extent that the nitrogen atom in the 3-position of the oxazoledione, hydantoin or rhodanine ring is quaternized and the sulfur atom in the 2-position is converted to a thioether group. In the second reaction (condensation), the alkylated trinuclear cyanine dye is condensed with a cyclammonium base or salt whereby symmetrical tetranuclear and new unsymmetrical tetranuclear cyanine dyes are obtained. Accordingly, the scope of my invention is to be limited solely by the appended claims.

I claim:

1. A photographic gelatino silver-halide emulsion containing a trinuclear cyanine dyestuff of the following general formula:



wherein m represents an integer of from 1 to 3, 65 R represents a member selected from the class consisting of hydrogen and lower alkyl groups, R being lower alkyl only when m represents 1, R<sub>1</sub> and R<sub>2</sub> represent a member selected from the class consisting of lower alkyl, allyl, aryl and aralkyl groups of the benzene and naphthalene series, R<sub>3</sub> represents a member selected from the class consisting of lower alkyl, lower hydroxy-alkyl, lower alkoxyalkyl, aryl and aralkyl groups of the benzene and naphthalene series, X represents an acid radical, Y represents the residue of a 5-membered heterocyclic nitrogenous ring

11

system, and Z represents the atoms necessary to complete a heterocyclic nitrogenous system.

2. A photographic gelatino silver-halide emulsion containing a trinuclear cyanine dyestuff of the following structure:



5

10

20

25

3. A photographic gelatino silver-halide emulsion containing a trinuclear cyanine dyestuff of the following structure:



5

10

20

25

12

4. A photographic gelatino silver-halide emulsion containing a trinuclear cyanine dyestuff of the following structure:



THOMAS R. THOMPSON.

No references cited.